

## UNITED STATES PATENT OFFICE

2,089,413

PRODUCTION OF NOVEL EFFECTS ON  
TEXTILES

Clifford Paine, Jack Augustus Radley, and Leslie  
Paige Rendell, Blackley, Manchester, England,  
assignors to Imperial Chemical Industries Lim-  
ited, a corporation of Great Britain

No Drawing. Application July 15, 1935, Serial No.  
31,522. In Great Britain July 18, 1934

9 Claims. (Cl. 8—6)

This invention relates to textile materials and a process of obtaining fluorescent effects thereon.

It is an object of the invention to produce novel effects on textiles whereby textiles although 5 colorless when illuminated by ordinary light are given the property of fluorescing when illuminated by ultra-violet light. A further object is to provide a process of producing valuable fluorescent properties on colored textiles dyed with 10 light-fast dyestuffs. An additional object is to produce new and improved textile materials which are colorless when viewed by ordinary light but give a colored fluorescence when illuminated by a source of relatively pure ultra-violet 15 light. Other objects will appear hereinafter.

According to the invention, we obtain fluorescent effects by subjecting a material to which has been applied a stilbene derivative, preferably an aminostilbene sulfonic acid, to a source of 20 relatively pure ultra-violet light. The stilbene derivative may be applied to the textile material by the methods generally used for applying acid 25 wool or direct cotton dyestuffs to textiles. For instance, we may apply to a textile fabric 4:4'-dibenzoyldiaminostilbene-2:2'-disulfonic acid or 25 a substitution derivative thereof, e. g., the p,p'-diamino derivative.

In practicing the invention we have found that the intensity of the fluorescent effect may vary 30 according to the nature of the stilbene derivative, the amount thereof and the type of textile material. Thus, we find that when 4:4'-dibenzoyldiamino- 35 stilbene-2:2'-disulfonic acid is applied to cotton, a fluorescent effect is obtained when 0.5% (on the weight of cotton) is used, and up to 3% may usefully be applied to cotton and other cellulose fibers, whilst on wool and animal fibers generally this compound has a very feeble effect. The compound 4:4'-di-p-aminobenzoyldiamino- 40 stilbene-2:2'-disulfonic acid gives on cotton a maximum fluorescent effect at about 0.1%. When as much as 5% is used, the fluorescence disappears. On wool and silk, however, up to 10% may be used but the fluorescence does not 45 vary in simple ratio with the amount of compound applied.

The invention is particularly valuable where cotton textiles are concerned, as will be seen from the following illustrative but not limitative examples.

## Example I

Three (3%) per cent of 4:4'-dibenzoyldiamino- 50 stilbene-2:2'-disulfonic acid, calculated on the weight of fiber, is applied to cotton yarn from

an aqueous bath containing 20% of Glauber salt. The usual methods of dyeing cotton with direct dyestuffs are followed. The temperature is kept at 80°-85° C. After forty-five minutes at this temperature, the yarn is lifted out, rinsed in 5 water and dried. It then shows a fine pale bluish fluorescence when illuminated by ultra-violet light, but in daylight it has the appearance of undyed bleached cotton.

10

## Example II

Cotton yarn is dyed as described in Example I with 1% of the direct cotton dyestuff known as Chlorazol Sky Blue FF (Color Index No. 518), together with 0.25% of 4:4'-di(p-aminobenzoylamino)-stilbene-2:2'-disulfonic acid.

The fabric so obtained has the normal shade of a fabric dyed with Chlorazol Sky Blue FF in daylight, but it is different in that it is brilliantly visible when illuminated by ultra-violet light, a 20 rich blue shade being seen.

## Example III

Woolen yarn is boiled for one hour in a liquor (50 parts to 1 part of wool) containing 0.5% of 25 4:4'-di(aminobenzoylamino)-stilbene-3:3'-disulfonic acid, calculated on the weight of yarn, and also 5% of acetic acid and 10% of Glauber's salt as is customary in dyeing some acid and direct 30 dyestuffs or wool. The yarn is mixed in water and dried. When viewed in daylight, it has the normal appearance of scoured wool but it shows strong fluorescence when illuminated by ultra-violet light.

Any suitable source of ultra-violet light may 35 be employed, as, for example, a mercury vapor lamp.

The invention is useful in obtaining spectacular stage effects. While it has heretofore been proposed to produce fluorescent effects on textiles, 40 the possibilities have been limited to the use of already colored textiles in the coloring of which otherwise unsatisfactory or not very satisfactory dyestuffs have been used. The present invention makes it possible to obtain colored fluorescent 45 effects on materials which in daylight have the appearance of undyed bleached cotton (compare Example I). It is also possible by this invention to obtain fluorescent effects on materials which are colored when viewed by daylight and wherein 50 the coloring is effected with a light-fast dye (compare Example II).

By the expression "aminostilbene sulfonic acid" as herein employed, we mean to include stilbene 55 compounds containing free amino groups and/or

substituted amino groups such as, for instance, acetyl amino, benzoyl amino and the like. We also mean to include compounds containing a single sulfonic acid group or a plurality of sulfonic acid groups.

As many apparently widely different embodiments of this invention may be made without departing from the spirit and scope thereof, it is to be understood that we do not limit ourselves to the specific embodiments thereof except as defined in the appended claims.

We claim:

1. A textile material containing a sufficient amount of an aminostilbene-sulfonic acid to be 15 fluorescent when subjected to ultra-violet light in the substantial absence of light in the visible portion of the spectrum.

2. A textile material containing a sufficient amount of a diaminostilbene-disulfonic acid to be 20 fluorescent when subjected to ultra-violet light in the substantial absence of light in the visible portion of the spectrum.

3. A textile material containing a sufficient amount of a dibenzoyldiaminostilbene-disulfonic 25 acid to be fluorescent when subjected to ultra-violet light in the substantial absence of light in the visible portion of the spectrum.

4. A textile material containing a sufficient

amount of 4:4'-dibenzoyldiaminostilbene-2:2'-disulfonic acid to be fluorescent when subjected to ultra-violet light in the substantial absence of light in the visible portion of the spectrum.

5. A textile material containing a sufficient 5 amount of 4:4'-di(p-aminobenzoyl amino)-stilbene-2:2'-disulfonic acid to be fluorescent when subjected to ultra-violet light in the substantial absence of light in the visible portion of the spectrum.

6. A textile material containing a sufficient amount of 4:4'-di(aminobenzoyl amino)-3:3'-disulfonic acid to be fluorescent when subjected to ultra-violet light in the substantial absence of light in the visible portion of the spectrum.

7. A cellulosic textile material containing about 15 0.5% to about 3% of 4:4'-dibenzoyldiaminostilbene-2:2'-disulfonic acid.

8. A cotton material containing about 3% of 4:4'-dibenzoyldiaminostilbene-2:2'-disulfonic 20 acid.

9. A cotton material containing about 0.1% to about 0.25% of 4:4'-di(p-aminobenzoyl amino)-stilbene-2:2'-disulfonic acid.

CLIFFORD PAINE.  
JACK AUGUSTUS RADLEY.  
LESLIE PAIGE RENDELL.

10

15

20

25